# EUROPEAN PATENT APPLICATION

(11) **EP 1 111 654 A1**
(43) Date of publication of application: **27.06.2001**
(21) Application number: 00311484.0
(22) Date of filing: 20.12.2000
(51) Int. Cl.: H01J 61/30, H01J 9/24

(54) **Single ended ceramic arc discharge lamp and method of making the same**

(30) Priority: 23.12.1999 US 471551
(71) Applicant: GENERAL ELECTRIC COMPANY, Schenectady, NY 12345 (US)
(72) Inventor: Scott, Curtis Edward, Mentor, Ohio 44060 (US); Boroczki, Agoston, 1157 Budapest (HU); Tambini, Antony John, Mountsorrel, Loughborough LE12 7HY (GB); Greskovitch, Charles David, Schenectady, New York 12309 (US); Preston, Barry, Ashby Rolville, Leicestershire LE14 2TE (GB)
(74) Representative: Pedder, James Cuthbert

(57) **Abstract**

A ceramic discharge lamp (20) includes first and second electrodes (24, 26) that are disposed in non-axial relation. In a preferred arrangement, the electrodes extend inwardly from one end of the lamp to define a single ended ceramic discharge lamp. The electrodes are disposed in parallel to provide for precise control of the arc gap in one exemplary embodiment while the electrodes are angled in non-parallel relation in another preferred embodiment to limit the potential for arcing outside of the chamber. The legs (62, 64) are integrally formed in one body component (60) and an integral lens is provided in the other body component to increase the lumens distribution since there is no leg to interfere with radiation from the chamber.

## Description

The present invention relates generally to lighting, and more particularly to a ceramic arc discharge lamp.

Discharge lamps produce light by ionizing a fill material such as a mixture of metal halides and mercury with an arc passing between two electrodes. The electrodes and the fill material are sealed within a translucent or transparent discharge chamber which maintains the pressure of the energized fill material and allows the emitted light to pass through it. The fill material, also known as a "dose", emits a desired spectral energy distribution in response to being excited by the electric arc. For example, halides provide spectral energy distributions that offer a broad choice of light properties, e.g., color temperatures, color renderings, and luminous efficacies.

Ceramic discharge lamp chambers were developed to operate at higher temperatures, i.e., above 950° C, for improved color temperatures, color renderings, and luminous efficacies, while significantly reducing reactions with the filler material. Typically, ceramic discharge chambers are constructed from a number of components which are extruded or die-pressed from a ceramic powder. Commonly owned, co-pending applications U.S. Serial No. 09/067,816, filed April 28, 1998 and U.S. Serial No. 09/250,634, filed February 16, 1999, describes one type of conventional ceramic discharge chamber which minimizes the number of joints used in forming the ceramic discharge chamber. For example, prior practice employed a five component construction including a central cylinder substantially closed at either end by first and second end plugs with first and second legs in the end plugs. The referenced application is directed to assemblies that use as few as two components to form the ceramic discharge chamber.

Commercially available ceramic metal halide lamp products all have at least one common feature. That is, each has a discharge tube geometry where the ceramic legs that receive the leads, the vacuum-tight ceramic-to-metal seals, and the electrodes are located at opposite ends of the discharge body. This standard double-ended ceramic discharge tube geometry is depicted in FIGURE 1. There are, however, instances where this geometry cannot satisfy the needs for a compact lamp structure. Thus, reducing the overall length of the lamp or the light center length and thereby increasing the compactness of the lamp designs has not been possible.

Reducing the length of the arc discharge tube in a standard double-ended discharge tube geometry as exhibited in Figure 1 still does not meet all of the needs of the industry. Reducing the discharge tube length is limited by the maximum temperature that the ceramic-to-metal seals at the ends of the ceramic legs can endure. Since the seal glass insures gas and vacuum tightness, designers have been careful to avoid exposing the seal to elevated or excess temperatures which may adversely affect the seal glass.

As is also described in the referenced co-pending application, limiting the number of components in the arc tubes and likewise the number of joints results in desired efficiencies and reduced manufacturing costs. Thus, eliminating manufacturing steps, components, and achieving improvements in the conductive and radiative heat losses with higher lamp efficacy are all desired features, while attaining better control on arc gap length results in flicker-free operation, more reliable starting, more stable operation, and increased lamp efficacy and color performance.

A ceramic discharge lamp includes a ceramic housing having a chamber adapted to receive a fill. First and second electrodes are disposed in spaced relation in the chamber to produce an arc in response to an electrical potential applied across the electrodes. The electrodes are disposed in non-axial relation relative to one another.

In an exemplary embodiment of the invention, the electrodes of the ceramic discharge lamp define a single-ended arc tube, i.e., the electrodes extend into the chamber from the same end of the arc tube.

Another preferred exemplary embodiment of the invention provides a dome-shaped end and optionally incorporates an integral lens therein.

Yet another exemplary embodiment angles the electrodes toward one another so that first ends disposed in the chamber are more closely dimensioned together than second ends disposed outside the chamber.

The invention will now be described in greater detail, by way of example, with reference to the drawings, in which:

FIGURE 1 illustrates a lamp assembly having a prior art ceramic discharge chamber.

FIGURES 2-13 are enlarged views of various ceramic arc discharge chambers according to exemplary embodiments of the invention.
FIGURE 1 illustrates a prior art ceramic discharge lamp **20** that includes a double-ended discharge chamber **22** which contains first and second electrodes **24, 26** and a fill material sealingly encapsulated in the discharge chamber. The electrodes **24, 26** are connected to conductors **28, 30** to apply a potential difference across the electrodes in a manner well know in the art. In operation, the electrodes produce an arc which ionizes the fill material to produce a plasma in the discharge chamber. For a ceramic metal halide lamp, the fill material typically includes a mixture of Hg, a rare gas such as Ar or Xe, and a metal halide such as Nal, Tll, or Dyl₃. Other examples of fill materials are well known in the art.

The discharge chamber includes a central cylindrical body portion **32** and first and second leg portions **34, 36**. The electrodes are connected to a power supply (not shown) by the conductors. The electrodes are typically constructed from tungsten, while the conductors are niobium and molybdenum since the thermal expansion coefficients are closely related to alumina to reduce thermally induced stresses on the alumina leg portions.

The discharge chamber is sealed at opposite ends as identified by reference numerals **40, 42**. The seals are preferably a dysprosia-alumina-silica glass frit received about the conductors and, when melted, the glass flows into the legs to form a seal between the conductor and leg. The dimensions of the leg portions are selected to reduce the temperature of the seals by a desired amount relative to the elevated temperature of the discharge chamber. As will be appreciated, the axial position of the electrodes affects the voltage drop across the electrodes which can have a significant effect on the quality of light produced. Thus, it is important to control the axial position of the legs since it effects the spacing between the electrodes.

As taught in the co-pending application identified above, it is desirable to reduce the number of components that comprise the discharge chamber to reduce the number of bonds between the components. This has the advantage of expediting assembly of the discharge chamber and reducing the number of potential bond defects during manufacture, as well as reducing the possibility of breakage of the discharge chamber at a bond region during handling. The components are preferably constructed by die-pressing a mixture of ceramic powder and a binder. For example, the mixture comprises 95 - 98 % by weight of ceramic powder and 2-5% by weight organic binder. The ceramic powder may comprise alumina (Al₂O₃) having a purity of 99.98% and a surface area of about 2-10m²/g. The alumina powder may be doped with magnesia to inhibit grain growth, for example in an amount equal to 0.03-0.2%, preferably 0.05%, by weight of the alumina. Other ceramic materials which may be used include non-reactive refractory oxides and oxynitrides, such as yttrium oxide, lutecium oxide, and hafnium oxide, and their solid solutions and compounds with alumina, such as yttrium-aluminum-garnet and alumina oxynitride. Binders which may be used individually or in combination include organic polymers such as polyols, polyvinyl alcohol, vinyl acetates, acrylates, cellulosics, and polyesters.

An exemplary composition which has been used for die pressing a solid cylinder comprises 97% by weight alumina powder having a surface area of 7 m²/g available from Baikowski International, Charlotte, NC, as Product Number CR7. The alumina powder was doped with magnesia in the amount of 0.1% of the weight of the alumina. The composition also comprised 2.5% by weight polyvinyl alcohol, available from GE Lighting as Product Number 115-009-018, and ½% (0.5%) by weight Carbowax 600, available from Interstate Chemical.

Subsequent to die pressing, the binder is removed from the green part, typically by thermal pyrolysis, to form a bisque-fired part. The thermal pyrolysis may be conducted, for example, by heating the green part in air from room temperature to a maximum temperature of about 900-1100° C over 4-8 hours, then holding the maximum temperature for 1-5 hours, and then cooling the part. After thermal pyrolysis, the porosity of the bisque-fired part is typically about 40-50%.

The bisque-fired part is then machined. For example, a small bore may be drilled along the axis of the solid cylinder which provides the bore of the first leg portion. Next, a larger diameter bore may be drilled along a portion of the axis to form the chamber. Finally, the outer portion of the originally solid chamber may be machined away along part of the axis, for example with a lathe, to form the outer surface of the first leg portion. The second leg member may be formed in a similar manner by first drilling a small bore which provides the bore through the leg portion, machining the outer portion of the originally solid cylinder to produce the leg portion and machining the transition portion, leaving the radially directed flange.

The machined parts are typically assembled prior to sintering to allow the sintering step to bond the parts together. According to an exemplary method of bonding, the densities of the bisque-fired parts used to form the body member and the leg are selected to achieve different degrees of shrinkage during the sintering step. The different densities of the bisque-fired parts may be achieved by using ceramic powders having different surface areas. For example, the surface area of the ceramic powder used to form a first component may be 6-10 m²/g, while the surface area of the ceramic powder used to form a second component may be 2-3 m²/g. The fine powder in the first component causes the bisque-fired body first component to have a smaller density than the bisque-fired second component made from the coarser powder. The bisque-fired density of the first component is typically 42-44% of the theoretical density of alumina (3.986 g/cm³), and the bisque-fired density of the second component is typically 50-60% of the theoretical density of alumina. Because the bisque-fired first component is less dense than the bisque-fired second component, relative shrinkage occurs (e.g., 3-10%) during sintering to form a seal around the transition. By assembling the two components prior to sintering, the sintering step bonds the two components together to form a discharge chamber.

The sintering step may be carried out by heating the bisque-fired parts in a refractory metal type furnace in hydrogen (H₂) with a dew point of about 0° C to +15° C at 1850° C for three to five hours. After heat treatment, the parts are cooled to room temperature over about two hours. The inclusion of magnesia in the ceramic powder typically inhibits the grain size from growing larger than 75 m. The resulting ceramic comprises a densely sintered polycrystalline alumina with optical translucency.

According to another method of bonding, a glass frit, e.g., comprising a refractory glass, can be placed between the first and second components to bond the two components together upon heating. According to this method, the parts can be sintered independently prior to assembly.

The first and second components typically each have a porosity of less than or equal to 0.1%, preferably less than 0.01%, after sintering. Porosity is conventionally defined as a unitless number representing the proportion of the total volume of an article which is occupied by voids. At a porosity of 0.1% or less, the alumina typically has a suitable optical transmittance or translucency. The transmittance or translucency can be defined as "total transmittance", which is the transmitted luminous flux of a miniature incandescent lamp inside the discharge chamber divided by the transmittance luminous flux from the bare miniature incandescent lamp. At a porosity of 0.1% or less, the total transmittance is typically 95% or greater.

According to another exemplary method of construction, the component parts of the discharge chamber are formed by injection molding a mixture comprising about 45-60% by volume ceramic material and 55-40% binder. The ceramic material can comprise an alumina powder having a surface area of about 1.5 to about 30 m²/g, typically between 3 - 5 m²/g. According to one embodiment, the alumina powder has a purity of at least 99.98%. The alumina powder may be doped with magnesia to inhibit grain growth, for example in an amount equal to 0.03 - 0.2%, preferably 0.05%, by weight of the alumina.

The binder may comprise a wax mixture or a polymer mixture. According to one example the binder comprises:
33α parts by weight paraffin wax, melting point 52-58° C;
33α parts by weight paraffin wax, melting point 59-63°;
33α parts by weight paraffin wax, melting point 73-80° C.

The following substances are added to the 100 parts by weight paraffin wax:
4 parts by weight white beeswax;
8 parts by weight oleic acid;
3 parts by weight aluminum stearate.
The above paraffin waxes are available from Aldrich Chemical, under Product Numbers 317659, 327212, and 411671, respectively.

In the process of injection molding, the mixture of ceramic material and binder is heated to form a high viscosity mixture. The mixture is then injected into a suitably shaped mold and subsequently cooled to form a molded part.

Subsequent to injection molding, the binder is removed from the molded part, typically by thermal treatment, to form a debindered part. The thermal treatment may be conducted by heating the molded part in air or a controlled environment, e.g., vacuum, nitrogen, rare gas, to a maximum temperature and then holding the maximum temperature. For example, the temperature may be slowly increased by about 2 - 3° C per hour from room temperature to a temperature of 160° C. Next, the temperature is increased by about 100° C per hour to a maximum temperature of 900 - 1100° C. Finally, the temperature is held at 900 - 1100° C for about 1 - 5 hours. The part is subsequently cooled. After the thermal treatment step the porosity is about 40 - 50%.

The bisque-fired parts are typically assembled prior to sintering to allow the sintering step to bond the parts together. Typically, the densities of the bisque-fired parts used to form the first and second components are selected to achieve different degrees of shrinkage during the sintering step. The different densities of the bisque-fired parts may be achieved by using ceramic powders having different surface areas, for example, as described above.

According to one example, an article was formed from a mixture comprising 48% by volume alumina and 52% by volume binder. The alumina had a surface area of 3 m²/g and was doped with magnesia in the amount of 0.05% of the weight of the alumina. The wax binder described above was used. The article, which had a thickness of about 3 mm, was sufficiently translucent that when pressed against newsprint, the newsprint could be read without difficulty through the article.

Without departing from the scope and intent of the present invention, it will be apparent to one in the field that other methods, such as machining-green or bisque fired ceramics, slip casting, and sol-gel processing may be used to manufacture and bond discharge chambers for use in ceramic discharge lamps.

With the general process of manufacture and bonding described above, or alternative processes, various single ended discharge chambers for use in ceramic discharge lamps will be described with reference to FIGURES 2-13. For example, FIGURES 2 and 3 illustrate first and second embodiments of a single ended ceramic discharge chamber which is a two component construction. The first component **50** includes a recess **52** that may be machined or formed as noted above. The continuous sidewall **54** provides a generally cylindrical configuration to the final conformation of the discharge chamber. A second component **60** includes first and second legs **62, 64,** respectively that extend therefrom. The legs are disposed in substantially parallel relation for reasons which will be noted below. They extend outwardly from a circular disk **66** which is dimensioned for receipt within the sidewall **54** of the first component. Once sintered and bonded together, the first and second components define a sealed ceramic arc discharge chamber having only one joint.

As a result of this geometry, the overall length of the discharge tube is considerably shorter than that illustrated in the double ended arrangements as exhibited in FIGURE 1. This leads to more compact lamp designs as a result of reducing the overall lamp length. In addition, the light center length dimensions are also reduced since both legs **62, 64** extend from one end of the arc discharge chamber. This can also be achieved without adversely impacting on the ceramic-to-metal seal that might otherwise be damaged due to the deleterious chemical reactions that are accelerated by excess temperature. That is, the seals in each of legs **62, 64** are disposed at a location remote from the chamber where the arc or plasma is operated at an elevated temperature. Additional advantages are also evident from this embodiment and the alternate embodiments described below. Particularly, more suitable light intensity distribution can be achieved. More luminous flux and light intensity distribution is attained since a clear end of the discharge tube is now provided. There is no longer an electrode or leg to interfere with the transmission of radiant energy from the non-leg end of the arc tube. The clear end of the discharge tube has a higher optical transmission so that discharge tube radiation and losses are reduced, and lamp efficacy and color performance increased.

Since only a single joint is used, the arc tube can be sealed in a single cycle, thereby eliminating manufacturing steps heretofore necessary for sealing purposes. Stated another way, this two piece arc tube arrangement with only one co-sintered joint maintains many of the advantages obtained in the co-pending application, while adding still further advantageous features.

Still another advantage is the ability to carefully control the arc gap dimension. The electrodes are not inserted from opposite ends of the arc discharge chamber such as in the prior art double-ended chambers where it is relatively difficult to control the desired arc gap. Instead, the single ended discharge tube configuration shown in FIGURE 2 defines the arc gap based on the parallelism of the ceramic legs. As will be appreciated, this arrangement is easier to control than the prior art to achieve a desired arc gap.

Still another consideration is that the single ended design would allow the electrodes to be sealed into the legs during sintering of the component. Moreover, the proposed single ended discharge tube geometry does not impose any constraints on the geometry of the plug or second component **60**. Again, and as referenced in the co-pending application, this permits the shape of the plug to be flat, spherical, cylindrical, or a mixture of these geometries. By carefully controlling the electrode design, flicker-free operation and a stable arc anchoring point location on the electrode surfaces can be assured.

FIGURE 3 illustrates a modification relative to FIGURE 2 wherein like components will be referenced by like reference numerals, and new components will identify new structural features. Here, the second component or plug includes a shoulder **70** that abuttingly engages a terminal end **72** of the sidewall **54** of the first component. This abutment provides a precise, positive axial location of the plug relative to the first component **50** of the ceramic arc discharge chamber.

The exemplary embodiment of FIGURE 4 slightly modifies the first component **80** so that it defines a plug having a shoulder **82** that provides positive axial location of the plug in an extended sidewall **84** of the second component. It will also be noted that the legs **62, 64** have portions **86, 88,** respectively, that extend inwardly into the chamber to achieve more reliable starting and more stable operation.

In FIGURE 5, an exhaust tube **90** is integrally formed in the first molded component or cover plug **80**. This illustrates the flexibility of the present design and the wide variation of modifications that can be advantageously incorporated into the design of the ceramic discharge chamber.

FIGURES 6 and 7 illustrate preferred embodiments employing differently shaped first components or cover members. In FIGURE 6, the cover member **100** has a generally dome-shape **102**. As will be appreciated, the member **100** is die-pressed or injection molded to provide a single ended discharge lamp design with a dome cover. The circumferentially continuous sidewall smoothly transitions or merges into the curved or dome shape. A shoulder **70** of the second component **60** abuttingly engages the terminal edge of the first component sidewall to from a single bond between the components. In FIGURE 7, the dome configuration includes an integral lens **104**. This, of course, enhances the light intensity distribution and result in more luminous flux being distributed as a result of a design specific lens being directly fabricated into the arc tube.

Variations of the single ended discharge chamber design are illustrated in FIGURES 8 and 9. When ultimately assembled, a single ended ceramic metal halide lamp having a compact design will be achieved. In these embodiments, however, the legs **110, 112** are formed in separate injection molded leg-plug components **114, 116**. These leg plug components are substantially identical except for the reverse or mirror image mating edges **118, 120**. This allows one of the leg plug components to shrink and form a sintered bond joint with the second leg-plug component. Each component includes a single leg integrally molded therein that precisely locates the electrode relative to each component. When brought together, these leg-plug components cooperate to define a complete single ended ceramic discharge chamber where the arc gap between the electrodes can be precisely dimensioned.

The concept is relatively similar in FIGURE 9, but includes a central body portion that may be formed, for example, from an extruded body **122**. Although the number of joints increases, it allows the central body component **122** to be formed, for instance, of an extruded Lucalox or alumina component. The same sintering and bonding steps described above achieve the desired joints at opposite ends of the central body with the individual leg-plug components. It also facilitates assembly if each leg plug component **114, 116** includes externally facing recesses **118** that are dimensioned for receipt within the opposite ends of the extruded body **122**.

As described above, certain advantages are achieved by using parallel legs to obtain a precise dimension between the electrodes, also known as the arc gap. FIGURES 10 and 11, on the other hand, illustrate advantages that may be offered by purposely angling the electrodes relative to one another. For example, in FIGURE 10, molded leg-plug-body component **130** includes legs **132, 134** that angle inwardly as they extend toward the discharge chamber. That is, the electrodes **136, 138** are positioned a predetermined dimension apart which is less than the dimension between the conductors **140, 142** at the outer ends of the legs. This arrangement prevents arcing between the leads at an area outside of the chamber. Since the distance between the leads is greater outside of the arc chamber, arcing is less likely to occur at that location as opposed to within the chamber as desired.

The preferred embodiment of FIGURE 11 also includes the angled electrode design. It further illustrates that other features can be incorporated into the ceramic arc discharge chamber design. Here, for example, the chamber interior includes curved recesses **150, 152**. As will be appreciated by one skilled in the art, such a configuration of the ceramic arc discharge chamber may be desirable in selected circumstances.

FIGURES 12 and 13 illustrate various combinations of the above described features. For example, in FIGURE 12, a dome-shaped cover **160** is used in conjunction with a second component **162** having a curved inner recess **164**. The legs are still defined in one component of the assembled discharge chamber so that all of the advantages of a single ended chamber are attained. This concept is slightly modified in FIGURE 13 where the legs include portions 166, 168 that extend inwardly into the discharge chamber. In substantially all other respects, however, the embodiment of FIGURE 13 is substantially similar to that in FIGURE 12.

The invention has been described with reference to the exemplary embodiments. Modifications and alterations will occur to others upon reading and understanding the specification. For example, the process and resultant material of U.S. Patent No. 4,285,732 can be used to produce an optically translucent alumina ceramic for use in association with the present invention.

For the sake of good order, various features of the invention are set out in the following clauses:-
1. A ceramic discharge lamp (20) comprising:
   a ceramic housing having a chamber (22) adapted to receive a fill therein; and first and second electrodes ( 24, 26) disposed in spaced relation in the chamber to produce an arc in response to an electrical potential applied across the electrodes, the electrodes disposed in non-axial relation relative to one another.
2. The ceramic discharge lamp of clause 1 wherein the ceramic housing is formed by injection molding.
3. The ceramic discharge lamp of clause 1 wherein the ceramic material comprises alumina.
4. The ceramic discharge lamp of clause 1 wherein the electrodes are disposed in substantially parallel relation relative to one another.
5. The ceramic discharge lamp of clause 1 wherein the electrodes (136, 138) are disposed in angled, non-parallel relation relative to one another.
6. The ceramic discharge lamp of clause 1 wherein the ceramic housing is formed from first and second body members (50, 60) bonded together.
7. The ceramic discharge lamp of clause 6 wherein the first and second body members (50, 60) are sintered together.
8. The ceramic discharge lamp of clause 6 wherein the first and second body members (50, 60) are bonded together along a single bond region.
9. The ceramic discharge lamp of clause 6 wherein the first and second electrodes (24, 26 ) both extend into the chamber from the first body member.
10. The ceramic discharge lamp of clause 9 wherein the second body member is formed into an integral lens (104).
11. The ceramic discharge lamp of clause 6 wherein the first and second electrodes extend into the chamber from the first and second body members , respectively.
12. A method of making a ceramic discharge chamber comprising the steps of:
   forming a first body member (50) from a ceramic material; forming a second body member (60) from a second ceramic material;
   orienting the first and second body members to define a chamber therebetween; and
   mounting first and second electrodes (24, 26) in non-axial relation relative to one another in at least one of the first and second body members.
13. The method of clause 12 further comprising the step of bonding the first and second body members (50, 60) together.
14. The method of clause 13 wherein bonding step includes sintering the first and second body members (50, 60) together.
15. The method of clause 12 wherein the mounting step includes mounting both the first and second electrodes in the first body member.
16. The method of clause 15 wherein the mounting step includes aligning the first and second electrodes in substantially parallel relation relative to one another.
17. The method of clause 15 wherein the mounting step includes orienting the first and second electrodes (136, 138) in angled relation relative to one another.
18. The method of clause 12 wherein the mounting step includes mounting the first electrode in the first body member and the second electrode in the second body member.
19. The method of clause 12 comprising the further step of integrally forming the second body member into a lens (104).

## Claims

1. A ceramic discharge lamp (20) comprising:
a ceramic housing having a chamber (22) adapted to receive a fill therein; and first and second electrodes ( 24, 26) disposed in spaced relation in the chamber to produce an arc in response to an electrical potential applied across the electrodes, the electrodes disposed in non-axial relation relative to one another.

2. The ceramic discharge lamp of claim 1 wherein the ceramic housing is formed by injection molding.

3. The ceramic discharge lamp of claim 1 or claim 2 wherein the ceramic material comprises alumina.

4. The ceramic discharge lamp of claim 1, 2 or 3 wherein the electrodes are disposed in substantially parallel relation relative to one another.

5. The ceramic discharge lamp of claim 1, 2 or 3 wherein the electrodes (136, 138) are disposed in angled, non-parallel relation relative to one another.

6. A method of making a ceramic discharge chamber comprising the steps of:
forming a first body member (50) from a ceramic material; forming a second body member (60) from a second ceramic material;
orienting the first and second body members to define a chamber therebetween; and
mounting first and second electrodes in non-axial relation relative to one another in at least one of the first and second body members.

7. The method of claim 6 further comprising the step of bonding the first and second body members together.

8. The method of claim 7 wherein bonding step includes sintering the first and second body members (50, 60) together.

9. The method of any one of claims 6 to 8 wherein the mounting step includes mounting both the first and second electrodes in the first body member.

10. The method of any one of claims 6 to 8 wherein the mounting step includes aligning the first and second electrodes in substantially parallel relation relative to one another.
